

## UNITED STATES PATENT OFFICE

1,955,927

## PROCESS OF MAKING PROPELLANT POWDERS

George A. McBride, Alton, Ill., assignor to  
Western Cartridge Company, East Alton, Ill., a  
corporation of Delaware

No Drawing. Application November 14, 1930  
Serial No. 495,672

14 Claims. (Cl. 52—20)

This invention relates to propellant powders, and more particularly powders of the type which are surface-treated with a deterrent to retard the initial combustion rates.

5 One of the objects of this invention is to provide a process of surface-treating propellant powders, and more particularly double base propellant powders adapted to improve the ballistic characteristics of such powders.

10 Another object is to provide a process of the character described whereby the application of the deterrent to the powder grain can be controlled to secure the desired application.

Another object is to provide a process whereby 15 the gravimetric density of a powder and more particularly a surface-treated powder, is increased, restored, or controlled.

Further objects will appear from the detail description, in which will be described an illustrative embodiment of this invention; it is to be understood however that this invention is susceptible of various other embodiments.

In the surface treatment of propellant powders with a deterrent, difficulty is experienced in 20 securing the desired uniform distribution of the deterrent on the powder grain, and it is especially difficult to secure uniformity of the application of the deterrent to the various grains of a batch. Moreover, since the deterrent employed 25 is usually a solvent or gelatinizer for the powder grain to be surface treated when the surfaces of the powder grains become softened through the action of the gelatinizing agent, the grains tend to stick together. These aggregates do not per-

30 mit the automatic volumetric measuring devices in the loading machines to operate satisfactorily so that variations in the weight of charge are encountered which give rise to erratic ballistic results. While a deterrent may be applied in a 35 solvent, difficulty is experienced in not only controlling the amount and penetration of the deterrent to be taken up by each grain, but where the vehicle employed is also a solvent for the powder grains these again tend to stick together.

40 Generally stated in accordance with this invention, the powder grains are treated with a deterrent while in a state of suspension. In accordance with one embodiment of this invention, the deterrent is emulsified with a suitable liquid 45 which is preferably a non-solvent for the powder grains; such a liquid is water, whereby a water emulsion of the deterrent can be made. In order to secure the addition of a predetermined amount of deterrent to powder grains, the powder grains 50 are treated with a predetermined amount of the

deterrent in the emulsified state until the deterrent is taken from the emulsion by the powder grain. In accordance with one embodiment of this invention, the powder grains are agitated in an emulsion of the deterrent and containing a 60 predetermined amount of the deterrent until the liquid with which the deterrent is emulsified clears. Where the deterrent is a liquid at ordinary temperatures, it can simply be mixed with, for instance, water, until an emulsion is secured; where, however, the deterrent is a solid at ordinary temperatures, it is heated to its melting point, either previous or after its addition to the liquid, such as water, and the treatment of the powder with emulsion is, therefore, carried out 65 at approximately the melting point of the deterrent. In such a case, after the liquid has cleared, additional liquid may be added and the agitation continued, however, at a reduced temperature.

70 In order to generally accomplish the objects of this invention, the deterrent may be one of the usual ones employed for that purpose. A deterrent which has been found particularly useful is diethyl-phthalate; a related deterrent, such as dibutyl-phthalate, may also be employed. Both, 75 of course, are active solvents for nitrocellulose and practically non-volatile. Moreover, waxes such as carnauba dinitro-toluene and the related mononitro and trinitro-toluenes may also be employed.

80 In the surface treatment of powder grains, and more particularly in the surface-gelatinizing of a powder with a deterrent, as heretofore described, it is found that the gravimetric density is decreased generally by the swelling of the surface of the grain to roughen or curl the same. This affects considerably the loading character of the powder and the amount which can be charged 85 into a shell of a given capacity. In accordance 90 with this invention, therefore, the powder is subjected to treatment for the purpose of restoring, increasing or controlling the gravimetric density so as to reduce the curl of the surfaces of the grains. This reduction of curl may be descriptively termed a smoothing of the general contour 95 of the grains although it will be understood that the surface irregularities need not be eliminated to accomplish this. This is accomplished in accordance with one embodiment of this invention 100 by treating the grains at a temperature and for a period sufficient, and in a suitable medium or vehicle such as water, so as to complete the gelatinization of the surfaces of the grains.

105 Many of the advantageous features of this invention may be secured by the surface treatment 110

of smokeless powder grains generally, when employing the process embodying this invention. This invention is, however, particularly applicable for the treatment of double base powders, such as nitro-cellulose-nitro-glycerin powders. A surface treated nitro-cellulose-nitro-glycerin powder grain which is of particular utility is one containing 15% nitro-glycerin and 5½% diamyl phthalate or 8-9% dinitro toluene.

10 As an illustrative embodiment of this invention, a nitro-cellulose-nitro-glycerine powder grain containing 15% nitro-glycerine is surface treated with diamyl phthalate in the following manner: A water emulsion is formed with the proper amount of the deterrent using, for instance, 5½ parts of the deterrent relative to 94½ parts of the powder. Into this emulsion the powder grains are dumped, agitation being continued until no cloudiness of the water is perceptible, that is, until the deterrent has been completely taken up by the powder grains. Because of the finely divided condition, almost colloidal, of the deterrent in the water, distribution is ideal, and the deterrent because of its efficient gelatinizing properties is attracted to the surfaces of the powder grains. As the deterrent droplets are picked up, the surface of the powder grains are softened; however, the presence of the water very efficiently cushions each grain from the others until gelatinization has been completed.

Where the gravimetric density of the powder has been decreased by the treatments heretofore described, the same is restored in the following manner: The powder is placed in water and held at 60° C. for about fifteen minutes. Upon drying it is found that the gravimetric density of, for instance, the nitro-cellulose-nitro-glycerine powder surface treated with D. A. P. is restored from .498 to .530. Upon storage for an extended period, this gravimetric density is not changed materially. The process is believed to be one of effecting complete gelatinization, thereby smoothing the contour of the grain to reduce its effective size.

45 Where the deterrent is dinitro toluene instead of diamyl phthalate, it is found that about twice the amount of deterrent is required. Now, DNT at ordinary temperatures is a solid; accordingly, the process is varied to the following extent: The amount of water required is heated to about 95° C. and the DNT allowed to melt in this water. Sufficient agitation is then applied to completely distribute the molten DNT throughout the water, so as to form an emulsion therewith. The powder when added very readily picks up the very tiny globules of DNT due perhaps to the accelerated gelatinization of nitro-cellulose at elevated temperatures. Agitation at this temperature is continued until the water is clear, which occurs in most cases between one and five minutes. Thereafter more water may be added or the container may be externally cooled so that the temperature is reduced to about 60° C. and agitation is continued at this temperature for about twenty-five minutes.

65 Whatever deterrent or process is employed, the water is easily removed by centrifuging and drying at the low temperature of 40° C. for approximately seventy-two hours. The powder grains when properly dried may be graphited and blended.

There is thus produced a powder grain, and more particularly a double base powder grain, which not only has the desired ballistic properties, but which can be made progressive burning

to the desired extent. It has been found that close control is possible with this process, and it has the further advantage in that it requires the use of no material which must be removed, except the water, which can be readily abstracted. Storage even at 50° C. carried out with this treated powder shows that it is remarkably stable. The process of restoring the gravimetric density is advantageous, for the charge which can be loaded into a shell of a given powder capacity can be increased to a maximum.

80 Powder prepared in accordance with the process embodying this invention is particularly suitable for small calibre rifle cartridges, in that it develops a maximum velocity with minimum pressures; thus when employed in 22 calibre "long rifle" cartridges, a mean charge of approximately 2.44 grains develops a mean velocity between 1200 and 1300 feet per second with a mean pressure of approximately 13,500 pounds per square inch.

85 In order to secure some of the advantageous features of this invention, the grains may be treated with a deterrent while in a state of suspension in a medium other than a liquid; thus the grains may be caused to pass through a dense 90 mist of a deterrent, such as diamyl phthalate, by generating such a mist by a spray of the heated deterrent. While this results in a rather efficient distribution of the deterrent over the powder grains, it is not as advantageous as where an 95 emulsion of the deterrent is employed; for in the latter, although the surfaces of the grains are softened by the deterrent, the presence of the liquid with which the deterrent is emulsified very efficiently cushions each grain from the others 100 until gelatinization has been completed, so that sticking together of the grains is avoided.

105 It will be understood that while this invention is particularly applicable to the treatment of double base powders, some of its features are of 110 advantage in the surface treatment of nitro-cellulose powders and smokeless powders generally. Furthermore, the process is not necessarily confined to the use of materials which melt below the boiling point of water because other substances which have a higher melting point can be conveniently used provided they are first dissolved in some suitable solvent. Instead of forming an emulsion using the melted deterrent at a 115 temperature near 100° C., it may be found convenient to first dissolve the deterrent in some 120 suitable solvent such as benzol. In this case an emulsion is then prepared comprising water as the continuous phase and the benzol solution of the wax or deterrent as the discontinuous phase. 125 It will further be understood that various features and subcombinations are of utility and may be employed without reference to other features and subcombinations; that is contemplated by and is within the scope of the appended claims. 130 It will be further understood that various changes may be made in details without departing from the spirit of this invention; it is, therefore, understood that this invention is not to be limited to the 135 specific details described.

140 Having thus described the invention, what is claimed is:

1. In the art of making propellant powders, the process comprising, treating powder grains with an emulsion of a solvent of low volatility.
2. In the art of making propellant powders, the process comprising, treating powder grains with a deterrent emulsified with a non-solvent for the powder grains.
3. In the art of making propellant powders, the

80

90

95

100

105

110

115

120

125

130

135

140

145

150

- process comprising, treating powder grains with a water emulsion of a deterrent. 80
4. In the art of making propellant powders, the process comprising, treating powder grains with an emulsion of a solvent of low volatility until the deterrent is taken from the emulsion by the powder grains. 85
5. In the art of making propellant powders, the process comprising, agitating powder grains in an emulsion of a solvent of low volatility. 90
6. In the art of making propellant powders, the process comprising, agitating powder grains with a predetermined amount of a deterrent emulsified with a liquid which is a non-solvent for the grains until the emulsion clears. 95
7. In the art of making propellant powders, the process comprising, treating powder grains with an emulsion of a deterrent approximate the melting point of the deterrent. 100
8. In the art of making propellant powders, the process comprising, agitating powder grains with a predetermined amount of a deterrent emulsified with a liquid until the emulsion clears, adding additional of the liquid and continuing the agita- 105
9. In the art of making propellant powders, the process comprising, agitating powder grains with a deterrent emulsified with a liquid approximate the melting point of the deterrent, adding additional liquid and continuing the agitation at a reduced temperature. 110
10. In the art of making propellant powders, the process comprising, treating powder grains with an emulsion of diamyl-phthalate. 115
11. In the art of making propellant powders, the process comprising, treating powder grains with an emulsion of dinitro-toluene. 120
12. In the art of making propellant powders, the process comprising, suspending a deterrent in a treating bath, and exposing powder grains to the action of the suspension. 125
13. In the art of making propellant powders, the process comprising, suspending a deterrent in a treating bath, exposing powder grains to the action of the suspension at a temperature approximate the melting point of the deterrent. 130
14. In the art of making propellant powders, the process comprising, suspending a solvent of low volatility in a treating bath, and exposing powder grains to the action of the suspension. 135

GEORGE A. McBRIDE.

- 30
- 35
- 40
- 45
- 50
- 55
- 60
- 65
- 70
- 75
- 105
- 110
- 115
- 120
- 125
- 130
- 135
- 140
- 145
- 150